

# United States Patent [19]

Van der Laan et al.

[11] 3,837,910

[45] Sept. 24, 1974

[54] METHOD OF MANUFACTURING A POLYCRYSTALLINE FERRITE BODY

[75] Inventors: **Karel Van der Laan; Hans Peter Peloschek**, both of Emmasingel, Eindhoven, Netherlands

[73] Assignee: **U.S. Philips Corporation**, New York, N.Y.

[22] Filed: **Oct. 4, 1971**

[21] Appl. No.: **186,254**

[30] Foreign Application Priority Data

Oct. 7, 1970 Netherlands ..... 7014697  
Aug. 18, 1971 Netherlands ..... 7111359

[52] U.S. Cl. .... **117/234, 252/62.58, 252/62.59, 252/62.6, 252/62.62, 252/62.63, 252/62.64, 264/60**

[51] Int. Cl. .... **C04b 35/30, C04b 35/38**

[58] Field of Search ..... **252/62.56-62.64; 117/100 B, 234; 264/60, 25, 27**

[56]

## References Cited

### UNITED STATES PATENTS

|           |         |                       |             |
|-----------|---------|-----------------------|-------------|
| 2,992,990 | 7/1961  | Parker .....          | 252/62.59 X |
| 3,002,930 | 10/1961 | Robinson et al. ....  | 252/62.62 X |
| 3,671,436 | 6/1972  | Peloschek et al. .... | 252/62.58   |

Primary Examiner—Jack Cooper

Attorney, Agent, or Firm—Frank R. Trifari; Carl P. Steinhauser

[57]

## ABSTRACT

A method of manufacturing a polycrystalline ferrite body obtained by sintering a compressed block of the starting material. A readily detrition-resistant material having interdigitated crystals of an average grain size of more than 50 microns is obtained by adding prior to sintering a material from the group  $\text{BaF}_2$ ,  $\text{SrF}_2$ ; the oxides of B, Bi, Ca, Cu, Mg, Pb, Si, V; and  $\text{Fe}_3(\text{PO}_4)_2$  and choosing a very particular combination of added quantity and sintering temperature.

4 Claims, 1 Drawing Figure

PATENTED SEP 24 1974

3,887,910



INVENTORS  
KAREL VAN DER LAAN  
HANS PETER PELOSCHEK

BY

Frank R. Siefen  
AGENT

**METHOD OF MANUFACTURING A  
POLYCRYSTALLINE FERRITE BODY**

The invention relates to a method of manufacturing a polycrystalline ferrite body, wherein a finely divided ferrite-forming starting mixture is formed, ground, pressed into a body having a desired shape and sintered.

A ferrite is to be understood to mean herein a crystalline reaction product of the oxides of iron and one or more other bivalent metals or bivalent metallic complexes.

Such a method is known from the U.S. Pat. No. 3,472,780.

As is known, bodies of sintered oxidic ferromagnetic material, for which material the name ferrite is generally used, are used inter alia as cores for electromagnetic transducers for converting electric signal variations into variations of the magnetic inductance, or conversely.

Since electromagnetic transducers, or magnetic heads, should cooperate in a number of applications in contact with a rapidly moving magnetic record carrier, for example a magnetic tape, the magnetic properties of the material and in particular the resistance to detrition, are of great importance. Two types of detrition are to be distinguished, the first type which is related to the hardness of the material used, manifests itself as a uniform "overall" reduction of the material of the contact surface of the transducer. The characteristics of the transducer in itself is not influenced by it. The second type which is inherent to the polycrystalline structure of the material used, manifests itself as a crumbling away of ferrite crystals out of the contact surface of the transducer under the influence of the scouring effect of the record carrier. When crystals crumble away at the edge of the effective gap, the rectilinearity thereof is lost and in circumstances the gap length, i.e., the dimension of the effective gap in the direction in which the record carrier moves relatively relative to the transducer, can be increased by it. It has been found actually that in the known regular crystal structures a crystal can crumble away comparatively easily along the boundary surface of the grain. Once in such a crystal structure one crystal has crumbled away, the surrounding crystals are supported and there is a fair chance that an increasing number of them starts crumbling away. The second type of detrition can therefore adversely influence the characteristic of the transducer.

This problem has been recognized in German Pat. No. 1,094,995 and the solution proposed in said patent specification as a core for a transducer which is to be readily resistant to crumbling away is the use of a ferrite body consisting of irregularly formed crystals which are as large as possible. In such a crystal structure the possibility of crumbling away of a crystal is much smaller since the irregularly formed and hence interdigitated crystals "hold" each other. It is proposed in particular in said patent specification to use a ferrite monocrystal as a core for a transducer. The manufacture of sufficiently large ferrite monocrystals, however, is expensive. Moreover, a drawback is that the resistance to detrition of the first type of monocrystals has been found to be not as large as that of polycrystalline material.

The invention provides a polycrystalline ferrite, having improved resistance to crumbling away. According to the invention a quantity of a material promoting grain growth or a combination of such materials chosen from the group consisting of  $\text{BaF}_2$ ,  $\text{SrF}_2$ , the oxides of B, Bi, Ca, Cu, Mg, Pb, Si, V and  $\text{Fe}_3(\text{PO}_4)_2$  is added to the ferrite-forming system during a manufacturing step preceding the sintering, such a combination of added quantity and sintering temperature being chosen, that interdigitated crystals of an average grain size of more than 50 microns are obtained.

In order to obtain a final product which as regards structure is as homogeneous as possible, according to a preferred embodiment of the method according to the invention the addition of the grain growth-promoting material or combination of such materials is made to the starting material to be ground. It is to be noted in that case the spreading in the average grain size may be very small, that is to say that so-called duplex structures do not occur.

In order to obtain a final product having magnetic and electrical properties which are favourable for its endeavoured application as a core for a magnetic head, the ferrite-forming starting mixture after grinding is preferably first pre-sintered and ground again before it is compressed to the desirable shape and sintered. In other words, a pre-sintered powder is used.

In order to obtain a final product having magnetic and electrical properties which are as favourable as possible, the method according to the invention may be varied so that the desirable crystal structure which is resistant to detrition occurs only at the surface or a part of the surface and that the internal structure is fine-granular which is a condition for good electric and magnetic properties. A further preferred embodiment of the method according to the invention is characterized in that the ferrite-forming starting mixture is compressed and pre-sintered, if desired, that the grain growth-promoting material or combination of materials is locally provided on the outside of the body obtained after compressing and possible pre-sintering, and that said body is then sintered.

In addition, the method according to the invention may also be varied so that the final product as such has a fine-granular structure but shows paths or patterns which consist of interdigitated crystals having an average grain size of more than 50 microns. Another preferred embodiment of the method according to the invention is therefore characterized in that the grain growth-promoting material or combination of materials is added to the starting mixture, that same is ground, compressed and presintered, and that the body obtained after compression and presintering is locally heated, during sintering, at a sintering temperature such that the desirable crystal structure occurs only at that region. Local heating to the sintering temperature can be realized, for example, by means of a laser beam or by means of a Pt-wire through which a current is conveyed.

Certain grain growth-promoting materials have turned out to be very effective within the scope of the present invention, provided the correct combination of added quantity and sintering temperature is found.

According to a further embodiment of the method according to the invention during the manufacture of a Ni-Zn ferrite body from 0.001 to 1 weight percent is added of the mixture determined by its molecular com-

position:  $x\text{B}_2\text{O}_3 + y\text{SiO}_2 + z\text{CaO}$ , with  $1 \leq x \leq 10$ ;  $0 \leq y \leq 10$ ;  $0 \leq z \leq 5$ , the sintering temperature lying between  $1,180^\circ\text{C}$  and  $1,275^\circ\text{C}$ .

It has been found that in this manner by means of the above-mentioned addition, a ferrite body can be obtained having interdigitated crystals with an average grain size of more than 50 microns. It is to be noted that the spreading in the average grain size can be very small. This means that so called "duplex structures" do not occur. It is furthermore to be noted that the magnetic and electrical properties of the ferrite bodies obtained in this manner are acceptable in all respects.

Although the above-mentioned addition provides the desirable crystal structure, attention should also be paid to other properties. For example, the crystal boundaries should be clean and comprise no large pores. This can be achieved by causing the addition to be 0.007 to 0.25 percent by weight of the starting mixture.

According to a preferred embodiment of the method according to the invention, the addition is characterized by the following molecular composition:  $2\text{B}_2\text{O}_3 + \text{SiO}_2$ , the sintering temperature lying between  $1,180^\circ\text{C}$  and  $1,240^\circ\text{C}$ . It has been found that, in particular after sintering of the compressed powder at a temperature between  $1,220^\circ\text{C}$  and  $1,230^\circ\text{C}$ , a product of maximum average grain size ( $> 500$  microns) can be obtained.

According to another preferred embodiment of the method according to the invention, the addition is characterized by the following molecular composition:  $\text{B}_2\text{O}_3 + 2\text{SiO}_2 + \text{CaO}$ .

It has been found that, after sintering of the compressed powder, a product can be obtained in which the average grain size does not or only slightly depends upon the sintering temperature used. It has been found in particular that variation of the sintering temperature between  $1,180^\circ\text{C}$  and  $1,275^\circ\text{C}$  has hardly any influence on the average grain size, although said temperature lies below the values found in the preceding case.

According to a further embodiment of the method according to the invention, the addition is characterized by the following molecular composition:  $\text{B}_2\text{O}_3 + 2\text{SiO}_2$  and the sintering temperatures lies between  $1,240^\circ\text{C}$  and  $1,300^\circ\text{C}$ . It has been found that, after sintering of the ground and compressed powder, a product is obtained having a combination of a high initial permeability  $\mu_i$  and a high density.

In manufacturing Ni-Zn ferrite bodies, the addition of  $\text{CaO} + \text{B}_2\text{O}_3$  has furthermore turned out to be very effective. According to a preferred embodiment of the method according to the invention from 0.01 to 0.2 percent by weight of  $\text{CaO} + \text{B}_2\text{O}_3$  is added during the manufacture of a Ni-Zn ferrite body and sintering takes place at a temperature between  $1,175^\circ\text{C}$  and  $1,250^\circ\text{C}$ , preferably between  $1,200^\circ\text{C}$  and  $1,250^\circ\text{C}$ .

Another preferred embodiment of the method according to the invention is characterized in that during the manufacture of a Ni-Zn ferrite body from 0.05 to 0.5 percent by weight of  $\text{BaF}_2$  and/or  $\text{SrF}_2$  is added and that sintering is carried out at the temperature between  $1,200^\circ\text{C}$  and  $1,250^\circ\text{C}$ .

Another preferred embodiment of the method according to the invention is characterized in that during the manufacture of a Ni-Zn ferrite body from 0.05 to 0.5 percent by weight of  $\text{BiF}_2\text{O}_3$  is added and that sintering is carried out at a temperature between  $1,175^\circ\text{C}$  and  $1,275^\circ\text{C}$ .

The addition of  $\text{CaO} + \text{B}_2\text{O}_3$  during the manufacture of Mn-Zn ferrite bodies has surprisingly been found to be even more effective than in the manufacture of Ni-Zn ferrite bodies, provided the correct sintering conditions where chosen.

Therefore, a preferred embodiment of the method according to the invention is characterized in that during the manufacture of a Mn-Zn ferrite body from 0.005 to 0.06 percent by weight of  $\text{CaO} + \text{B}_2\text{O}_3$  is added and that sintering is carried out in an oxygen-containing atmosphere at a temperature between  $1,350^\circ\text{C}$  and  $1,400^\circ\text{C}$ .

A further preferred embodiment of the method according to the invention is characterized in that during the manufacture of a Mn-Zn ferrite body from 0.005 to 1 percent by weight of the mixture  $x\text{B}_2\text{O}_3 + y\text{SiO}_2 + z\text{Fe}_3(\text{PO}_4)_2$  wherein  $0 \leq x \leq 1$ ;  $0 \leq y \leq 1$ ;  $0 \leq z \leq 1$  determined by its molecular composition is added and that sintering is carried out in an oxygen-containing atmosphere at a temperature between  $1,350^\circ\text{C}$  and  $1,400^\circ\text{C}$ .

Still a further preferred embodiment of the method according to the invention is characterized in that during manufacture of a Mn-Zn ferrite body from 0.005 to 0.5 percent by weight of  $\text{BaF}_2$  is added and that sintering is carried out in an oxygen-containing atmosphere at a temperature between  $1,350^\circ\text{C}$  and  $1,400^\circ\text{C}$ .

Another further preferred embodiment of the method according to the invention is characterized in that during the manufacture of a Mn-Zn ferrite body from 0.005 to 0.05 percent by weight of  $\text{V}_2\text{O}_5$  is added and that sintering is carried out in an oxygen-containing atmosphere at a temperature between  $1,375^\circ\text{C}$  and  $1,400^\circ\text{C}$ .

The invention also relates to a sintered oxidic ferromagnetic body manufactured by using one or more of the above-mentioned methods.

The invention will now be described with reference to the drawing and to the following examples.

#### EXAMPLE 1

To ferrite-forming systems of the composition

49.50 – 49.99 mol percent  $\text{Fe}_2\text{O}_3$ ,

$\text{NiO}$  and  $\text{ZnO}$  according to the proportion 18 : 32 was added a series of additions (0.01 percent by weight, 0.81 percent by weight and 1 percent by weight) of grain growth promoting materials.

Each of the resulting mixtures was pre-ground for 6 hours in a ball mill which also contained a grinding liquid and then prefired in oxygen at a temperature of  $850^\circ\text{C}$  for 3 hours. The mixtures were then post-ground for 16 hours. The powders obtained in this manner (grain size from 0.1 to a few microns) were precompressed to blocks at a pressure of  $10\text{ kg per cm}^2$  and post-compressed in an isostatic pressure vessel at a pressure of  $1,000\text{ kg/cm}^2$ . The compressed product was sintered for 24 hours at temperatures of  $1,180^\circ\text{C}$ ,  $1,200^\circ\text{C}$ ,  $1,225^\circ\text{C}$ ,  $1,250^\circ\text{C}$  and  $1,275^\circ\text{C}$ , respectively, in a furnace containing an oxygen-containing atmosphere, for example air or a relatively more oxygen-containing atmosphere. The heating time was 16 hours and the cooling time was 24 hours.

The resulting products were polished and etched at one of their surfaces so as to evaluate their crystal

structure. An average crystal size was determined with reference to microphotographs by dividing the distance covered during traversing by the number of crystal boundaries which is passed during covering said distance, in which of course the magnification standard should be taken into account.

while said material in addition shows a very regular crystal structure. The average grain size of the material manufactured by means of the method according to the invention turns out to be at least a factor 10 higher while the crystals are shaped very whimsically and are interdigitated.

TABLE I

| (molecular)<br>composition<br>of the<br>addition | % by weight | sintering temperature, (°C) |      |      |      |      |
|--------------------------------------------------|-------------|-----------------------------|------|------|------|------|
|                                                  |             | 1180                        | 1200 | 1225 | 1250 | 1275 |
| 1. $B_2O_3$                                      | 0.01        | 154                         | 256  | 120  | 164  | 256  |
|                                                  | 0.1         | 111                         | 272  | 246  | 113  | 62   |
| 2. $2B_2O_3 + SiO_2$                             | 0.01        | 271                         | 230  | 679  | 104  | 37   |
|                                                  | 0.1         | 85                          | 124  | 153  | 119  | 124  |
| 3. $B_2O_3 + SiO_2$                              | 0.01        | 124                         | 365  | 136  | 129  | 176  |
|                                                  | 0.1         | 76                          | 82   | 100  | 95   | 95   |
| 4. $B_2O_3 + 2SiO_2$                             | 0.01        | 19                          | 18   | 23   | 165  | 250  |
|                                                  | 0.1         | 85                          | 95   | 102  | 119  | 160  |
| 5. $B_2O_3 + 2SiO_2 + CaO$                       | 0.01        | 17                          | 21   | 26   | 28   | 40   |
|                                                  | 0.1         | 144                         | 127  | 130  | 131  | 137  |
| 6. $SiO_2 + CaO$                                 | 0.01        | 10                          | 10   | 11   | 13   | 21   |
|                                                  | 0.1         | 70                          | 76   | 71   | 68   | 54   |
| 7. $B_2O_3 + CaO$                                | 0.01        | 2                           | 34   | 112  | 153  | 161  |
|                                                  | 0.1         | —                           | 23   | 83   | 95   | 75   |
| 8. $Fe_3(PO_4)_2$                                | 0.01        | —                           | 110  | 110  | 154  | 84   |
|                                                  | 0.1         | —                           | 23   | 33   | 36   | 17   |
| 9. $B_2O_3 + SiO_2 + Fe_3(PO_4)_2$               | 0.01        | 76                          | 40   | 64   | 58   | 55   |
|                                                  | 0.1         | 27                          | 25   | 21   | 26   | 29   |
| 10. $BaF_2$                                      | 0.01        | 45                          | 31   | 29   | 43   | 47   |
|                                                  | 0.1         | 45                          | 52   | 68   | 77   | 54   |
| 11. $SrF_2$                                      | 0.01        | 19                          | 17   | 15   | 17   | 25   |
|                                                  | 0.1         | 7                           | 13   | 15   | 16   | 14   |
| 12. $CaF_2$                                      | 0.01        | 13                          | 16   | 18   | 24   | 28   |
|                                                  | 0.1         | 11                          | 13   | 16   | 21   | 32   |
| 13. $PbO$                                        | 0.01        | 17                          | 20   | 20   | 28   | 35   |
|                                                  | 0.1         | 17                          | 12   | 23   | 24   | 29   |
| 14. $Bi_2O_3$                                    | 0.01        | 15                          | 17   | 19   | 22   | 19   |
|                                                  | 0.1         | 93                          | 92   | 81   | 100  | 90   |
|                                                  | 1           | 36                          | 43   | 30   | 26   | 50   |

When:

A = distance in centimeters traversed on the photograph,

S = magnification standard (1 cm = . . . microns)

N = number of counted crystal boundaries,

$\bar{\delta}$  = average cross-section of a crystal in microns,

$$\text{then } \bar{\delta} = A/NxS \text{ (microns).}$$

The average grain sizes found in this manner are represented in Table I as a function of the addition and of the sintering temperature for a sintering time of 24 hours.

On the basis of this table, an expert can adapt a distinct material to his specific wishes.

For comparison the average grain size of NiZn-ferrite manufactured in the usual manner is 10 to 20 microns,

It is to be noted that the sintered products obtained by using the method according to the invention show magnetic and electric values which are acceptable in all respects for the end in view. The following example demonstrates this: Addition of 0.01 percent by weight  $(B_2O_3 + SiO_2)$ , sintering temperature 1,180° C, gives a product with a density 5.305 g/ccm, and a  $\mu_i = 1,160$ ; and an addition of 0.01 percent by weight  $(B_2O_3 + 2SiO_2)$ , sintering temperature 1,250° C, gives a product with a density of 5.310 g/ccm and a  $\mu_i = 1,700$ . (The X-ray density for these compositions is 5.336 g/ccm).

A series of more extensive investigations were carried out on ferrite-forming systems to which  $CaO + B_2O_3$  had been added. The results of these tests are shown by the FIGURE which represents the average grain size (in microns) as a function of the added quantity in percent by weight and of the sintering temperature T. It is obvious that a maximum average crystal growth (250  $\mu$ ) is obtained with a very particular combination of sintering temperature and added quantity.

It is to be noted that the result shown is characteristic of the behaviour of the grain growth-promoting materials mentioned further in this application.

It is furthermore to be noted that dependent upon the reactivity of the relevant ferrite-forming mixture (which is determined by the nature and the quality of the raw materials), the system of lines shown in the drawing of equal average grain size can slightly shift as a whole relative to the axes.

### EXAMPLE II

A similar series of experiments as in Example I was carried out in ferrite-forming systems of the following composition:

52.75 mol %  $\text{Fe}_2\text{O}_3$

22 mol %  $\text{ZnO}$

25.25 mol %  $\text{MnO}$ .

The starting mixture was treated in the same manner as in Example I. This means that each mixture was pre-ground in a ball mill for 6 hours and than pre-fired in air at a temperature of  $850^\circ\text{C}$  for 4 hours. The mixture was then post-ground for 6 hours. The powders obtained in this manner were pre-compressed to blocks at a pressure of 10 kg/sq.cm and post-compressed in an

isostatic pressure vessel at a pressure of 1,000 kg/sq.cm.

The compressed blocks were then sintered, in which the range of sintering temperatures, however, as chosen to be higher than in Example I, namely from  $1,200^\circ$  to  $1,400^\circ\text{C}$ .

The average grain sizes measured in the final products are recorded in Table II as a function of the nature and quantity of the addition and of the sintering conditions.

Condition A means that sintering was carried out at a temperature of  $1,300^\circ\text{C}$  in air for 2 hours.

Condition B means that sintering was carried out at a temperature of  $1,370^\circ\text{C}$  in 100 percent oxygen for 5 hours so as to obtain the desirable crystal structure.

Condition C means that sintering was carried out at a temperature of  $1,390^\circ\text{C}$  in 100 percent oxygen for 5 hours so as to obtain the desirable crystal structure.

In the cases B and C, afterfining may then be carried out at a lower temperature (for example,  $1,290^\circ\text{C}$ ) for a few hours (for example 3 hours) in an atmosphere containing 0.1 percent oxygen so as to adjust the ferro-ferrite equilibrium, after which conditioned cooling may be carried out, for example, in a nitrogen atmosphere.

TABLE II

|    | molecular composition of the addition                               | % by weight                  | sintering condition           |                               |     |
|----|---------------------------------------------------------------------|------------------------------|-------------------------------|-------------------------------|-----|
|    |                                                                     |                              | A                             | B                             | C   |
| 1  | $\text{B}_2\text{O}_3$                                              | 0.01<br>0.1<br>1             | 785<br>287<br>50              | 22<br>23<br>69.910            |     |
| 2  | $\text{CaO} + \text{B}_2\text{O}_3$                                 | 0.01<br>0.1<br>1             | 828<br>16<br>24-300           | 16-500<br>56<br>24            |     |
| 3  | $\text{SiO}_2 + \text{CaO}$                                         | 0.01<br>0.1<br>1             | 26<br>81<br>24-300            | 24<br>16<br>16                |     |
| 4  | $\text{B}_2\text{O}_3 + \text{SiO}_2$                               | 0.01<br>0.1<br>1             | 828<br>169<br>44              | 16<br>14<br>211               |     |
| 5  | $\text{B}_2\text{O}_3 + 2\text{SiO}_2$                              | 0.01<br>0.1<br>1             | 648<br>240<br>61              | 710<br>481<br>339             |     |
| 6  | $2\text{B}_2\text{O}_3 + \text{SiO}_2$                              | 0.01<br>0.1<br>1             | 764<br>153<br>37              | 931<br>219<br>48              |     |
| 7  | $\text{B}_2\text{O}_3 + 2\text{SiO}_2 + \text{CaO}$                 | 0.1<br>1<br>0.01<br>0.1<br>1 | 282<br>22<br>481<br>255<br>68 | 373<br>22<br>784<br>23<br>117 |     |
| 8  | $\text{B}_2\text{O}_3 + \text{SiO}_2 + \text{Fe}_3(\text{PO}_4)_2$  | 0.01<br>0.1<br>1             | >1000<br>166<br>17            | 23<br>226<br>89               |     |
| 9  | $\text{B}_2\text{O}_3 + 2\text{SiO}_2 + \text{Fe}_3(\text{PO}_4)_2$ | 0.1<br>1                     | 994<br>368<br>114             | >1000<br>355<br>144           |     |
| 10 | $2\text{B}_2\text{O}_3 + \text{SiO}_2 + \text{Fe}_3(\text{PO}_4)_2$ | 0.01<br>0.1<br>1             | 311<br>40-1000<br>22-450      | 21<br>105<br>321              |     |
| 11 | $\text{Fe}_3(\text{PO}_4)_2$                                        | 0.1<br>1                     | 96<br>710<br>269              | 1240<br>269<br>68             |     |
| 12 | $\text{BaF}_2$                                                      | 0.01<br>0.1<br>1             | 17<br>14<br>304               | 620<br>211<br>47              |     |
| 13 | $\text{SrF}_2$                                                      | 0.01<br>0.1<br>1             | 24<br>17<br>35                | 23<br>66<br>48                |     |
| 14 | $\text{CdF}_2$                                                      | 0.01<br>0.1<br>1             | 18<br>281<br>382              | 23-180<br>22-450<br>22-500    |     |
| 15 | $\text{Bi}_2\text{O}_3$                                             | 0.01<br>0.1<br>1             | 17<br>347<br>261              | 26<br>21<br>24                |     |
| 16 | $\text{PbO}$                                                        | 0.01<br>0.1<br>1             | 23<br>27<br>22                | 19<br>174<br>271              |     |
| 17 | $\text{CuO}$                                                        | 0.01<br>0.1<br>1             | 18<br>22<br>9                 | 18<br>19<br>19                |     |
| 18 | $\text{MgO}$                                                        | 0.01<br>0.1<br>1             | 172                           | 22<br>9                       | 207 |

TABLE II—Continued

| molecular<br>composition<br>of the<br>addition | % by weight | sintering condition |     |   |
|------------------------------------------------|-------------|---------------------|-----|---|
|                                                |             | A                   | B   | C |
| 19 $V_2O_5$                                    | 0.01        | 25                  | 745 |   |
|                                                | 0.1         | 27                  | 331 |   |
|                                                | 1           | 56                  | 29  |   |
| 20                                             | 0           | 18                  | 24  |   |
|                                                | 0           | 21                  | 22  |   |
|                                                | 0           | 22                  | 18  |   |

## EXAMPLE III

A number of investigations were carried out on Ni-Zn ferrite samples on the surface of which a thin 15 layer was provided (vapour-deposited or coated) of the crystal growth-promoting materials mentioned in the preceding examples, after which the samples were sintered at temperatures which varied from 1,200° to 1,250° C and for periods of time which varied from 20 to 24 hours.

One half of the investigated samples were manufactured by grinding a (Ni-Zn) ferrite-forming mixture for 6 hours, presintering it at a temperature of 850° C in an oxygen-containing atmosphere for 3 hours, post-grinding for 16 hours, pre-compressing, isostatic post-compressing at a pressure of 100 kg/sq.cm, after which a layer of grain growth-promoting material was provided, and sintering for 24 hours in oxygen at a temperature of 1,240° C. Samples manufactured in this manner turned out to yield no useful result.

The other half of the samples was manufactured by grinding a (Ni-Zn) ferrite-forming mixture for 6 hours, pre-sintering for 3 hours, post-grinding, pre-compressing and isostatically post-compressing at a 35 pressure of 1,000 kg/sq.cm, after which a layer of grain growth-promoting material was provided on the surface. When the material to be provided is available in powder form, it can be provided directly on the compressed body. When the material is available in a liquid form, it is to be preferred to pre-sinter the compressed body slightly so that a denser structure is obtained.

The desired crystal structure occurred without an exception after providing each of the above-mentioned grain growth-promoting materials followed by sintering. When using the materials CuO; CaO+SiO<sub>2</sub>; SrF<sub>2</sub>; BaF<sub>2</sub>, the desired crystal structure turned out to be restricted most to the surface and the least deformation of the surface also occurred.

## EXAMPLE IV

A number of detrition experiments was carried out both in magnetic heads of — normal — Ni-Zn ferrite having regularly shaped crystals and an average grain size of from 10 to 20 microns, and in magnetic heads 55 manufactured from Ni-Zn ferrite having interdigitated crystals having an average grain size of more than 50 microns manufactured while using the method according to the invention.

Commercially available magnetic tape (Kodak p 300 M; BASF-PES 18) were used for these experiments and

conducted along the heads at an increased tape speed of 38 cms per second. The frequency characteristic was determined at regular instants and the product recorded by means of the relevant head was subjected to a quality evaluation.

The life of heads manufactured from a material manufactured while using the method according to the invention turned out in the examined case to be twice more favourable and, when using the same reject criteria, it turned out to be even a factor 3 more favourable.

| Material                     | Life Head  |
|------------------------------|------------|
| regularly formed             |            |
| $\bar{s} = 10$ to 20 microns | 1500 hours |
| irregularly formed           |            |
| $\bar{s} > 50$ microns       | 4500 hours |

What is claimed is:

1. A method of manufacturing a detrition-resistant polycrystalline ferrite body comprising the steps of forming a finely-divided mixture of iron oxide, zinc oxide, and an oxide selected from the group consisting of nickel and manganese in proportions forming upon heating at an elevated temperature a nickel- or manganese-zinc ferrite, forming a body of said mixture, covering said body with a material promoting grain growth and selected from the group consisting of BaF<sub>2</sub>, SrF<sub>2</sub>, an oxide selected from the group consisting of B, Bi, Ca, Cu, Mg, Pb, Si, V, and Fe<sub>3</sub>(PO<sub>4</sub>)<sub>2</sub>, and thereafter sintering said body in an oxygen-containing atmosphere at a temperature of about 1,180° to 1,400°C to form a coherent ferrite body having a surface structure of interdigitated crystals of an average grain size of more than 50 microns.

2. A method as claimed in claim 1 in which the body is formed by compacting and pre-sintering said mixture at a temperature of about 850°C.

3. A method as claimed in claim 2 in which the material promoting grain growth is applied in liquid form.

4. A method as claimed in claim 1 in which the body is compacted by compression and the material promoting grain growth applied to the thus compacted body.

\* \* \* \* \*

UNITED STATES PATENT OFFICE  
CERTIFICATE OF CORRECTION

Patent No. 3,837,910 Dated September 24, 1974

Inventor(s) KAREL VAN DER LAAN ET AL

It is certified that error appears in the above-identified patent  
and that said Letters Patent are hereby corrected as shown below:

Column 1, line 47 after "supported" insert --less--;  
Column 2, line 12, after "regards" insert --crystal--.

Signed and sealed this 10th day of June 1975.

(SEAL)

Attest:

RUTH C. MASON  
Attesting Officer

C. MARSHALL DANN  
Commissioner of Patents  
and Trademarks